

## UNITED STATES PATENT OFFICE

EDWARD A. TAYLOR, OF CLEVELAND, OHIO, ASSIGNOR, BY MESNE ASSIGNMENTS, TO KREBS PIGMENT & COLOR CORPORATION, OF WILMINGTON, DELAWARE, A CORPORATION OF DELAWARE

## PROCESS OF MAKING LITHOPONE WITH HIGH ZINC SULPHIDE CONTENT

No Drawing.

Application filed January 23, 1928. Serial No. 248,974.

The term lithopone designates usually the white pigment obtained by calcining a mixture of co-precipitated zinc sulphide and barium sulphate in which the components 5 are present in substantially equimolecular proportions.

It is well known in this art that one essential feature of the process of making this pigment consists in producing the two components 10 simultaneously and from the same reaction medium, and the standard practice of the precipitation step in making lithopone consists in effecting double decomposition between water solutions of equimolecular 15 amounts of zinc sulphate and barium sulphide.

While this regular lithopone has for a long time met all the requirements of the trade, it was found that by increasing the zinc sulphide content of such a pigment over that corresponding to the equimolecular proportion improves considerably the covering power 20 of the lithopone. In this case again it is essential that the two components be co-precipitated. These lithopones of high zinc sulphide content are commonly called superlithopones, and for convenience sake this term as used herein is meant to designate lithopones containing more than 1 and not more 25 than 2 molecular equivalents of zinc sulphide to 1 of barium sulphate.

My invention consists now in a process of co-precipitating a mixture of zinc sulphide and barium sulphate in which the molecular 30 ratio of zinc sulphide to barium sulphate ranges from 1:1 to 2:1. This process consists substantially in reacting in aqueous solutions upon zinc sulphate with a barium sulphide compound in which the amount of 35 available  $S^{2-}$  ions is greater than that of the  $Ba^{2+}$  ions. The barium sulphide compounds corresponding to the above definition are barium hydrosulphide and mixtures of barium sulphide with barium hydrosulphide.

40 As will be seen from the formula  $Ba(SH)_2$ , barium hydrosulphide has 2 available  $S^{2-}$  ions against 1  $Ba^{2+}$  ion, whereas in barium sulphide  $BaS$ , or if written to correspond to the usual conception of aqueous barium sulphide solutions:  $(Ba(SH)_2 + Ba(OH)_2)$ ,

there will be the same amount of  $Ba^{2+}$  and  $S^{2-}$  ions, and in mixtures of the sulphide and hydrosulphide a proportionately higher amount of  $S^{2-}$  ions against  $Ba^{2+}$  ions will be present.

55 The amount of zinc sulphate used should preferably be adjusted to be substantially equivalent to that of the  $S^{2-}$  ions as there will otherwise be a waste of material which cannot react and is lost.

60 In taking the extreme case of barium hydrosulphide the chemical reactions involved can be represented by the formula:



65 This reaction equation would appear to be partly reversible as the free sulphuric acid could react with the zinc sulphide formed. I have, however, found that a substantially complete precipitation of this zinc sulphide 70 can be effected if the concentration of the free sulphuric acid in the reaction medium is kept at about  $\frac{1}{2}\%$  or below. It will be necessary when working in higher concentrated solutions to neutralize all of, or at least the 75 sulphuric acid in excess of that corresponding to the above limit concentration. The most convenient neutralizing agents which I can use are the carbonates and bicarbonates of the alkali metals; they do not form insoluble sulphates which would be precipitated together with the zinc sulphide and barium sulphate 80 and contaminate the finished lithopone.

85 It is evident from the above that by using 1 molecular equivalent of zinc sulphate and 1 molecular equivalent of barium hydrosulphide, a co-precipitated mixture of 1 equivalent of barium sulphate and 2 equivalents of zinc sulphide will be obtained, or, in other words, the finished superlithopone will have 90 substantially the composition 45.5%  $ZnS$  plus 54.5%  $BaSO_4$ ; this compares with the regular lithopone which has the theoretical composition 29.5%  $ZnS$  plus 70.5%  $BaSO_4$ .

95 When a lithopone of a composition intermediate between the above limits is desired, I replace part of the barium hydrosulphide by barium sulphide, and in this manner decrease the amount of  $S^{2-}$  ions available for the precipitation of the zinc sulphide.

The reaction equation can then be expressed by the following:



5 The values of  $x$  in this formula must, of course, be greater than  $y$  and not greater than  $2y$ .

I am aware that for theoretical reasons it is generally considered that barium sulphide 10 in aqueous solutions exists in a form corresponding to the equilibrium



The two components on the right hand 15 side of this equation are, however, not separable and for all practical purposes, particularly the co-precipitation of zinc sulphide and barium sulphate, the barium sulphide liquor reacts exclusively as if it contained 20 only BaS; as a matter of fact, whatever molecular proportions of barium sulphide and zinc sulphate are allowed to react upon each other, the co-precipitated zinc sulphide and barium sulphate will always appear in equi- 25 molecular proportion.

The most convenient procedure for performing my invention is to dissolve the requisite amount of zinc sulphate in water, heat the solution to about 180° F., slowly add 30 thereto the barium hydrosulphide solutions, adding simultaneously the calculated amount of neutralizing agent which, when using soda ash, is added solid and in successive small amounts. It is in this manner very easy to 35 maintain the reaction mixture faintly alkaline to phenolphthalein or slightly acid, as desired. It is well known that certain properties of the subsequently obtained lithopone can be controlled by adjusting the acidity or 40 alkalinity of the reaction mixture during the co-precipitation of the zinc sulphide and barium sulphate.

Similarly, in producing superlithopones of from above 30 to about 45% zinc sulphide 45 content, a hot aqueous solution containing the predetermined calculated amounts of barium hydrosulphide and barium sulphide is slowly run into the heated zinc sulphate solution with gradual addition of the neutralizing agent.

The precipitated zinc sulphide and barium sulphate is then filtered off and the green cake dried, calcined and worked up. This part of the lithopone manufacturing process 55 is in no way different when using the superlithopone green cake of my invention, and as it is well known by these skilled in this art and is no part of my invention, need not be described in detail.

60 The above procedure was substantially followed in the examples given below, which will further illustrate my invention; the parts given therein are by weight:

(1). 696 parts zinc sulphate solution containing 31.44% zinc sulphate were heated to

about 180° F. and a hot mixture of 213 parts barium hydrosulphide solution containing 20% Ba(SH)<sub>2</sub> and 1030 parts barium sulphide solution containing 15.4% BaS slowly introduced, 35 parts soda ash being simultaneously added. 70

The reagents used are in the proportion 1.44 mols. ZnSO<sub>4</sub>, 0.22 mols. Ba (SH)<sub>2</sub>, 1 mol. BaS, and 0.35 mols. Na<sub>2</sub>CO<sub>3</sub>. The calcined superlithopone had a composition of 30.78% 75 ZnS, 0.11% ZnO and 67.75% BaSO<sub>4</sub>.

(2). Similarly, the following reagents were used:

1.75 mols. ZnSO<sub>4</sub>, 0.38 mols. Ba (SH)<sub>2</sub>, 1 mol. BaS, and 0.38 mols. Na<sub>2</sub>CO<sub>3</sub>. The 80 finished superlithopone contained 32.9% ZnS, 0.08% ZnO, and 64.8% BaSO<sub>4</sub>, and had very desirable coloristic as well as physical properties.

(3). 450 parts barium sulphide liquor containing 15.4% BaS, 627 parts barium hydrosulphide liquor containing 20% Ba(SH)<sub>2</sub>, 845 parts zinc sulphate liquor containing 31.44% ZnSO<sub>4</sub> and 65 parts soda ash were reacted and the precipitated superlithopone 90 green cake calcined as usual after thorough working.

The finished product had a composition of 38.6% ZnS, 0.09% ZnO, and 60.0% BaSO<sub>4</sub>.

(4). 950 parts barium hydrosulphide 95 liquor containing 20% Ba(SH)<sub>2</sub> were at 150° F. slowly run into 960 parts zinc sulphate liquor containing 31.44% ZnSO<sub>4</sub> and 98.8 parts soda ash gradually added. The green cake was again washed and calcined as usual. 100

The finished superlithopone contained 42.6% ZnS and 55.75% BaSO<sub>4</sub>.

It will be apparent from the above that the zinc sulphide in the superlithopone is slightly deficient when compared with the amount expected from the reaction equation. This is partly due to the use of more or less impure, technical products, and also to the well known and difficultly avoidable formation of zinc oxide and other insoluble zinc compounds during the finishing of the lithopone. 110

I claim:

1. In a process of making a super-lithopone the step comprising co-precipitating zinc sulphide and barium sulphate by reacting upon an aqueous zinc sulphate solution with an aqueous solution of a barium sulphide compound in which the amount of available S<sup>-</sup> ions is substantially greater than the amount of available Ba<sup>++</sup> ions, the amounts of the reacting ingredients being so chosen that the amount of available Zn<sup>++</sup> ions is substantially greater than the said amount of Ba<sup>++</sup> ions. 115

2. In a process of making a super-lithopone the step comprising co-precipitating zinc sulphide and barium sulphate by reacting upon an aqueous zinc sulphate solution with an aqueous solution of a barium sulphide compound in which the amount of available 120

S<sup>2-</sup> ions is substantially greater than the amount of available Ba<sup>++</sup> ions, the amounts of reacting ingredients being so chosen that the amount of available Zn<sup>++</sup> ions is substantially equivalent with said amount of S<sup>2-</sup> ions and substantially greater than said amount of Ba<sup>++</sup> ions, and neutralizing the free sulphuric acid produced by a neutralizing agent, the sulphate of which is water soluble.

15 3. In a process of making a superlithopone the step comprising co-precipitating zinc sulphide and barium sulphate by reacting in aqueous solution upon substantially 2 molecular equivalents of zinc sulphate with substantially 1 molecular equivalent of barium hydrosulphide and neutralizing the free sulphuric acid formed by gradual addition of soda ash to the reaction mixture.

20 In testimony whereof, I affix my signature.  
EDWARD A. TAYLOR.

25

30

35

40

45

50

55

60

65